

[54] CORROSION-RESISTANT ALLOYS

[75] Inventor: John H. Culling, Kirkwood, Mo.

[73] Assignee: Carondelet Foundry Company, St. Louis, Mo.

[22] Filed: Sept. 24, 1973

[21] Appl. No.: 399,687

[52] U.S. Cl. .... 75/134 F, 75/122, 75/134 C

[51] Int. Cl. .... C22c 31/00

[58] Field of Search ..... 75/134 F, 134 C, 122, 171

[56] References Cited

UNITED STATES PATENTS

|           |         |                  |        |
|-----------|---------|------------------|--------|
| 2,860,968 | 11/1958 | Boegehold et al. | 75/122 |
| 2,938,786 | 5/1960  | Johnson          | 75/171 |
| 3,758,294 | 9/1973  | Bellot et al.    | 75/122 |
| 3,758,296 | 9/1973  | Johnson          | 75/122 |
| 3,759,704 | 9/1973  | Culling          | 75/122 |

FOREIGN PATENTS OR APPLICATIONS

36,659 11/1970 Japan ..... 75/134 F

Primary Examiner—L. Dewayne Rutledge

Assistant Examiner—E. L. Weise

Attorney, Agent, or Firm—Koenig, Senniger, Powers and Leavitt

[57] ABSTRACT

A workable, machinable alloy having good corrosion resistance to sulfuric acid solutions over a wide range of acid concentrations. The alloy consists essentially of between about 35.2 and about 46.2 percent by weight nickel, between about 14.9 and about 25.3 percent by weight chromium, between about 6.7 and about 14.5 percent by weight molybdenum, between about 4.3 and about 8.1 percent by weight copper, between about 14.06 and about 30.62 percent by weight iron, up to about 1.50 by weight manganese, up to about 0.11 percent by weight carbon, up to about 1.00 percent by weight silicon, up to about 0.010 percent by weight boron, up to about 1.00 percent by weight niobium, up to about 2.00 percent by weight tantalum, and up to about 1.00 percent by weight titanium. It is also essential that the sum of the molybdenum content and copper content be at least about 11.7 percent by weight. The sum of the niobium plus one-half the tantalum content should not exceed about 1.00 percent by weight.

4 Claims, No Drawings

## CORROSION-RESISTANT ALLOYS

## BACKGROUND OF THE INVENTION

This invention relates to the field of corrosion-resistant alloys and particularly to novel alloys suitable for use with a wide range of sulfuric acid concentrations.

Not only are sulfuric acid solutions very corrosive generally, but the nature of their corrosive properties varies markedly with both acid concentration and temperature. In most concentration ranges, sulfuric acid solutions are strong reducing acids. In higher concentrations, however, and particularly at elevated temperatures, sulfuric acid solutions can be oxidizing and in some instances highly oxidizing.

As a consequence of this variability in the corrosive properties of sulfuric acid, few materials are available which are reasonably resistant to sulfuric acid solutions over a wide range of concentrations. A relatively large number of available materials exhibit reasonable resistance to either dilute sulfuric acid solutions having an acid strength of less than about 20 percent by weight or to concentrated solutions having acid strengths of greater than 80 percent by weight. A lesser number of materials are effective for the intermediate and generally more corrosive concentration range of 20 to 80 percent; and even fewer metal alloys are commercially useful in contact with sulfuric acid solutions ranging from strengths below 20 to greater than 80 percent, particularly when exposed to elevated temperatures.

Of the known alloys which are demonstratedly effective over wide ranges of sulfuric acid concentrations, many contain relatively high proportions of nickel and are thus rather expensive. Many of such alloys are relatively brittle and cannot be readily machined or wrought, and are thus suitable only for use in castings which need not be machined.

## SUMMARY OF THE INVENTION

Among the several objects of the present invention, therefore, may be noted the provision of alloys which are resistant to sulfuric acid solutions over a wide range of acid concentrations; the provision of such alloys which retain good corrosion-resistant properties at elevated temperatures; the provision of such alloys which are resistant under conditions which may become highly oxidizing; the provision of alloys which may be readily machined and wrought; and the provision of alloys which may be formulated at moderate cost. Other objects and features will be in part apparent and in part pointed out hereinafter.

The present invention is therefore directed to a corrosion-resistant alloy consisting essentially of between about 35.2 and about 46.2 percent by weight nickel, between about 14.9 and about 25.3 percent by weight chromium, between about 6.7 and about 14.5 percent by weight molybdenum, between about 4.3 and about 8.1 percent by weight copper, between about 14.06 and about 30.62 percent by weight iron, up to about 0.11 percent by weight carbon, up to about 1.00 percent by weight silicon, up to about 1.50 percent by weight manganese, up to 0.010 percent by weight boron, up to about 1.00 percent by weight niobium, up to about 2.00 percent by weight tantalum, and up to about 1.00 percent by weight titanium. The sum of the molybdenum content and the copper content is at least about

11.7 percent by weight, while the sum of the niobium content and one-half the tantalum content is no greater than about 1.00 percent by weight.

## DESCRIPTION OF THE PREFERRED EMBODIMENTS

The alloys of the present invention exhibit highly satisfactory corrosion resistance in sulfuric acid solutions ranging from 10 by weight to 93 percent by weight and higher. The high resistance of these alloys is maintained at elevated temperatures, for example 176°F. and under conditions which are highly oxidizing. Good corrosion resistance is also exhibited by these alloys under the strongly de-passivating effect of chloride ions, for example, in hydrochloric acid solutions at room temperature. The alloys of the invention, moreover, have advantageous mechanical properties and can be rolled, drawn, machined or otherwise worked in accordance with conventional forming and fabricating techniques.

While the alloys possess outstanding corrosion resistance properties, their formulation cost is moderate. The proportions of iron which can be tolerated in these alloys are high enough to allow the use of ferro alloys for their formulation. The essential components of the alloys of the invention are:

| Per cent By Weight |                 |                |
|--------------------|-----------------|----------------|
| 30                 | Nickel          | 35.2 to 46.2   |
|                    | Chromium        | 14.9 to 25.3   |
|                    | Molybde-<br>num | 6.7 to 14.5    |
| 25                 | Copper          | 4.3 to 8.1     |
|                    | Iron            | 14.06 to 30.62 |

A critical parameter of the alloys of the invention is the sum of the molybdenum and copper content, which must be at least about 11.7 percent by weight. A synergistic effect of copper and molybdenum on the corrosion resistance of the alloys is realized when the total concentration of copper plus molybdenum exceeds 11.7 percent by weight.

Various other components are optionally present in the alloys of the invention, and the presence of certain of these components is advantageous especially for certain particular applications.

| Per cent By Weight |           |                  |
|--------------------|-----------|------------------|
| 50                 | Carbon    | Up to 0.11       |
|                    | Silicon   | Up to 1.00       |
|                    | Manganese | Up to 1.50       |
| 55                 | Boron     | Up to 0.010      |
|                    | Niobium   | Up to 1.00       |
|                    | Tantalum  | Up to about 2.00 |
|                    | Titanium  | Up to about 1.00 |

The sum of the niobium and one-half of the tantalum content generally should not exceed about 1.00 percent by weight.

The presence of a small proportion of boron, for example, about 0.005 percent by weight is desirable where workability of the alloy is particularly important. The presence of up to 0.010 percent by weight boron enhances elongation values and hence workability. The presence of up to 1.50 percent by weight manganese also contributes to the workability of the alloy.

Up to 1.00 percent by weight titanium, or niobium plus one-half the tantalum, may be included to eliminate the need for solution heat treatment of the alloys following welding, casting or cold working. Titanium, niobium and tantalum are effective for stabilizing carbide which may otherwise cause intergranular corrosion in alloys which are not heat treated subsequent to welding. Where carbide stabilization is important, the alloys preferably contain at least 10 parts by weight niobium plus tantalum or at least five parts by weight titanium per one part by weight carbon. Titanium, niobium and tantalum also have a beneficial effect upon fabricability.

tent, and a corresponding lower allowable iron content than the alloys of this invention. Moreover, most Illium alloys are rather brittle and hard and are not as susceptible to machining and cold working as are the alloys of the present invention.

5 The following examples illustrate the invention.

#### EXAMPLE 1

10 100-lb. heats of seven different alloys were prepared in accordance with the invention. Each of these heats was dead-melted in a 100-lb. high frequency induction furnace. The composition of these alloys is set forth in Table I.

Table I

| Alloy No. | Percent by Weight of Alloying Elements |       |       |      |      |     |      |      |     |       | Iron, By Difference |
|-----------|----------------------------------------|-------|-------|------|------|-----|------|------|-----|-------|---------------------|
|           | Ni                                     | Cr    | Mo    | Cu   | C    | Si  | Mn   | B    | Ti  |       |                     |
| 1         | 36.44                                  | 14.94 | 12.32 | 8.06 | .04  | .53 | .39  | —    | —   | 27.28 |                     |
| 2         | 38.01                                  | 18.25 | 14.51 | 5.91 | .11  | .61 | .48  | —    | —   | 22.12 |                     |
| 3         | 37.54                                  | 18.19 | 9.66  | 7.01 | .076 | .54 | .47  | —    | —   | 26.51 |                     |
| 4         | 35.24                                  | 20.84 | 12.74 | 5.18 | .10  | .71 | .50  | —    | —   | 24.69 |                     |
| 5         | 35.70                                  | 19.94 | 6.90  | 4.81 | .04  | .97 | 1.02 | .005 | 1.0 | 30.62 |                     |
| 6         | 38.23                                  | 20.73 | 6.74  | 5.58 | .04  | .92 | 1.08 | .005 | 1.0 | 26.68 |                     |
| 7         | 46.17                                  | 25.28 | 8.32  | 4.37 | .05  | .72 | 1.03 | .005 | 1.0 | 14.06 |                     |

High ductility and superior fabricability properties are achieved if the alloy composition falls within the following preferred range:

|                     |                                  |
|---------------------|----------------------------------|
| Nickel              | 35.70% to 46.17%                 |
| Chromium            | 18.19% to 25.28%                 |
| Molybdenum          | 6.74% to 9.66%                   |
| Copper              | 4.37% to 7.01%                   |
| Carbon              | 0.11% maximum                    |
| Molybdenum + Copper | 11.71% minimum to 16.67% maximum |
| Silicon             | 1.00% maximum                    |
| Manganese           | Up to 1.50% maximum              |
| Niobium + Tantalum  | 10 × Carbon to 1.00% maximum     |
| Titanium            | 5 × Carbon to 1.00% maximum      |
| Iron                | 14.06% to 30.62%                 |

45 It will be noted that these preferred alloys are also especially economical to formulate because of the relatively low proportions of molybdenum which they contain. Molybdenum is the most expensive of the elements of which these alloys are constituted. The relatively high proportions of chromium contained by these preferred alloys also promotes good corrosion resistance to a wide variety of corrosive media.

The corrosion resistance of the alloys of the invention compares favorably with that of other commercially available alloys designed for use in sulfuric acid, including, for example, alloys such as those sold under the Illium trade designation. The Illium alloys, which are adapted for use over a wide range of sulfuric acid concentrations, have a higher "critical element" con-

30 30 Standard physical test blocks and corrosion test bars were prepared from each heat. The mechanical properties of each of these alloys was then measured in the as-cast state. The results of these measurements are set forth in Table II.

Table II

| Alloy No. | Mechanical Properties |                          |                        |              |
|-----------|-----------------------|--------------------------|------------------------|--------------|
|           | Brinell Hardness      | Tensile Strength, P.S.I. | Yield Strength, P.S.I. | % Elongation |
| 1         | 152                   | 47,430                   | 35,450                 | 5.0          |
| 2         | 187                   | 56,090                   | 42,750                 | 4.0          |
| 3         | 148                   | 57,880                   | 37,040                 | 18.5         |
| 4         | 193                   | 58,640                   | 46,760                 | 2.5          |
| 5         | 149                   | 45,520                   | 34,320                 | 10.0         |
| 6         | 167                   | 55,770                   | 38,430                 | 14.5         |
| 7         | 207                   | 61,407                   | 39,440                 | 24.0         |

40 40 The corrosion test bars were annealed for 30 minutes at 1,950°F. and oil-quenched prior to machining into 1½ inch diameter by ¼ inch high discs having a ½ inch diameter hole in the center. Care was exercised during machining to obtain an extremely smooth surface on the discs. Twelve to fourteen discs were obtained for each alloy.

55 55 These discs were used in the comparative corrosion tests described hereinafter, comparing the performance of the alloys of the invention with a number of commercially available alloys. The compositions of the commercially available alloys which were used in these tests and the respective trade designations under which they are marketed are set forth in Table III.

Table III

| Alloy        | Commercial Alloys Utilized in Comparative Corrosion Tests |    |     |     |     |     |     |      |     |      | Iron, By Difference |
|--------------|-----------------------------------------------------------|----|-----|-----|-----|-----|-----|------|-----|------|---------------------|
|              | Ni                                                        | Cr | Mo  | Cu  | C   | Si  | Mn  | B    | Ti  |      |                     |
| Carpenter 20 | 29                                                        | 20 | 2.3 | 3.3 | .05 | .50 | .95 | —    | —   | 44.  |                     |
| No.20Cb3     | 33                                                        | 20 | 2.3 | 3.3 | .05 | .50 | .95 | .005 | 1.0 | 39.6 |                     |
| PH55A        | 9                                                         | 20 | 4.0 | —   | .04 | 3.5 | .5  | —    | —   | 63.  |                     |

Table III -Continued

| Commercial Alloys Utilized in Comparative Corrosion Tests |    |      |     |      |     |      |      |    |    |                     |
|-----------------------------------------------------------|----|------|-----|------|-----|------|------|----|----|---------------------|
| Alloy                                                     | Ni | Cr   | Mo  | Cu   | C   | Si   | Mn   | B  | Ti | Iron, By Difference |
| PH55B                                                     | 9  | 20   | 5.0 | 3.5  | .04 | 1.5  | .5   | —  | —  | 61.                 |
| PH55C                                                     | 9  | 20   | 4.0 | 3.0  | .04 | 3.5  | .5   | —  | —  | 60.                 |
| 316 Stainless                                             | 12 | 20   | 2.5 | —    | .05 | .8   | .7   | —  | —  | 64.                 |
| Illiump G                                                 | 56 | 22.5 | 6.4 | 6.5  | .20 | .65  | 1.25 | —  | —  | 6.5                 |
| Illiump 98                                                | 55 | 28   | 8.5 | 5.5  | .05 | .90  | 1.25 | —  | —  | 1.                  |
| Illiump B                                                 | 50 | 28   | 8.5 | 5.5  | .05 | 5.5  | 1.25 | .5 | —  | 2.5                 |
| CD4MCu                                                    | 5  | 25   | 2   | 3    | .03 | .5   | .5   | —  | —  | 64.                 |
| Worthite                                                  | 24 | 20   | 3.0 | 1.75 | .07 | 3.50 | 1.00 | —  | —  | 46.7                |

## EXAMPLE 2

Comparative corrosion tests were run in 10 percent by weight sulfuric acid solution at 176°F.

Disc samples of Carpenter 20, Carpenter 20Cb3, Cooper PH55A, Cooper PH55B, Cooper PH55C, CD4MCu, Worthite, 316 Stainless Steel, Illiump G, Illiump 98, and 304 Stainless Steel were prepared in the manner described in Example 1. Residual machining oil and dirt were removed from all of the sample discs by cleaning them with a small amount of carbon tetrachloride. The discs were then rinsed in water and dried.

Each disc was weighed to the nearest 10,000th of a gram and then suspended in a beaker by a piece of thin plastic wire hooked through the center hole of the disc and attached to a glass rod which rested on top of the beaker. Sufficient 10 percent sulfuric acid solution was then added to the beaker so that the entire sample was immersed. The temperature of the acid was thermostatically controlled at 176°F. by means of a water bath, and each beaker was covered with a watch glass to minimize evaporation.

After precisely 6 hours, the sample discs were removed from the sulfuric acid solution and cleaned of corrosion products. Most samples were cleaned sufficiently with a small nylon bristle brush and tap water. Those samples on which the corrosion product was too heavy for removal with a nylon brush were cleaned with a 1-to-1 solution of hydrochloric acid and water. After the corrosion products had been removed, each disc was again weighed to the nearest 10,000th of a gram. The corrosion rate of each disc, in inches per year, was calculated by the following formula in accordance with ASTM specification G1-67.

$$R_{ipy} = 0.3937 (W_o - W_f) / ATD$$

where

$R_{ipy}$  = corrosion rate in inches per year

$W_o$  = original weight of sample

$W_f$  = final weight of sample

$A$  = area of sample in square centimeters

$T$  = duration of test in years

$D$  = density of alloy in g./cc.

Results of this corrosion test are set forth in Table IV.

## Table IV

| CORROSION RATES IN 10% $H_2SO_4$ AT 176°F. (80°C.) |                                                   |  |
|----------------------------------------------------|---------------------------------------------------|--|
| Alloy No.                                          | Losses in Inches of Penetration Per Year (I.P.Y.) |  |
| 1                                                  | 0.0038                                            |  |
| 2                                                  | 0.0008                                            |  |

## Table IV-Continued

| CORROSION RATES IN 10% $H_2SO_4$ AT 176°F. (80°C.) |                                                   |
|----------------------------------------------------|---------------------------------------------------|
| Alloy No.                                          | Losses in Inches of Penetration Per Year (I.P.Y.) |
| 3                                                  | 0.0030                                            |
| 4                                                  | 0.0027                                            |
| 5                                                  | 0.0049                                            |
| 6                                                  | 0.0022                                            |
| 7                                                  | 0.0016                                            |
| Carpenter 20                                       | 0.005                                             |
| No. 20Cb3                                          | 0.0045                                            |
| PH55A                                              | 0.023                                             |
| PH55B                                              | 0.0006                                            |
| PH55C                                              | 0.00012                                           |
| CD4MCu                                             | 0.004                                             |
| Worthite                                           | 0.030                                             |
| 316 Stainless                                      | 0.197                                             |
| Illiump G                                          | 0.0051                                            |
| Illiump 98                                         | .003                                              |
| 304 Stainless                                      | 4.5                                               |

## EXAMPLE 3

Comparative tests were conducted in 25 percent sulfuric acid solution at 176°F. Sample discs were prepared and tested in the manner described in Example 2, except that a 25 percent sulfuric acid solution was used in place of the 10 percent sulfuric acid solution. The results of this test are set forth in Table V.

## Table V

| CORROSION RATES IN 25% $H_2SO_4$ AT 176°F. (80°C.) |                                                   |
|----------------------------------------------------|---------------------------------------------------|
| Alloy No.                                          | Losses in Inches of Penetration Per Year (I.P.Y.) |
| 1                                                  | 0.0143                                            |
| 2                                                  | 0.0025                                            |
| 3                                                  | 0.0005                                            |
| 4                                                  | 0.0116                                            |
| 5                                                  | 0.0000                                            |
| 6                                                  | 0.0000                                            |
| 7                                                  | 0.0000                                            |
| Carpenter 20                                       | 0.010                                             |
| No. 20Cb3                                          | 0.010                                             |
| PH55A                                              | 0.055                                             |
| PH55B                                              | 0.050                                             |
| PH55C                                              | 0.015                                             |
| CD4MCu                                             | 0.200                                             |
| Worthite                                           | 0.020                                             |
| 316 Stainless                                      | >0.200                                            |
| Illiump G                                          | 0.004                                             |
| Illiump 98                                         | 0.007                                             |

## EXAMPLE 4

Comparative tests were conducted in 40 percent sulfuric acid solution at 176°F. Sample discs were prepared and tested in the manner described in Example 2, except that a 40 percent sulfuric acid solution was

used in place of the 10 percent sulfuric acid solution. The results of this test are set forth in Table VI.

Table VI

| CORROSION RATES IN 40% H <sub>2</sub> SO <sub>4</sub> AT 176°F. (80°C.) |                                                   |
|-------------------------------------------------------------------------|---------------------------------------------------|
| Alloy No.                                                               | Losses in Inches of Penetration Per Year (I.P.Y.) |
| 1                                                                       | 0.0021                                            |
| 2                                                                       | 0.0027                                            |
| 3                                                                       | 0.0022                                            |
| 4                                                                       | 0.0062                                            |
| 5                                                                       | 0.0011                                            |
| 7                                                                       | 0.0000                                            |
| Carpenter 20                                                            | 0.016                                             |
| No. 20Cb3                                                               | 0.009                                             |
| PH55A                                                                   | 0.11                                              |
| PH55B                                                                   | >0.1                                              |
| PH55C                                                                   | >0.1                                              |
| Worthite                                                                | 0.019                                             |
| Illium G                                                                | 0.0062                                            |
| Illium 98                                                               | 0.0054                                            |

EXAMPLE 5

Comparative tests were conducted in 50 percent sulfuric acid solution at 176°F. Sample discs were prepared and tested in the manner described in Example 2, except that a 50 percent sulfuric acid solution was used in place of the 10 percent sulfuric acid solution. The results of this test are set forth in Table VII.

Table VII

| CORROSION RATES IN 50% H <sub>2</sub> SO <sub>4</sub> AT 176°F. (80°C.) |                                                   |
|-------------------------------------------------------------------------|---------------------------------------------------|
| Alloy No.                                                               | Losses in Inches of Penetration Per Year (I.P.Y.) |
| 1                                                                       | 0.0000                                            |
| 2                                                                       | 0.0000                                            |
| 3                                                                       | 0.0027                                            |
| 4                                                                       | 0.0019                                            |
| 5                                                                       | 0.0016                                            |
| 6                                                                       | 0.0000                                            |
| 7                                                                       | 0.0103                                            |
| Carpenter 20                                                            | 0.017                                             |
| No. 20Cb3                                                               | 0.008                                             |
| PH55B                                                                   | >0.1                                              |
| PH55C                                                                   | >0.1                                              |
| Worthite                                                                | 0.029                                             |
| Illium G                                                                | 0.005                                             |
| Illium 98                                                               | 0.005                                             |

EXAMPLE 6

Comparative tests were conducted in 60 percent sulfuric acid solution at 176°F. Sample discs were prepared and tested in the manner described in Example 2, except that a 60 percent sulfuric acid solution was used in place of the 10 percent sulfuric acid solution. The results of this test are set forth in Table VIII.

Table VIII

| CORROSION RATES IN 60% H <sub>2</sub> SO <sub>4</sub> AT 176°F. (80°C.) |                                                   |
|-------------------------------------------------------------------------|---------------------------------------------------|
| Alloy No.                                                               | Losses in Inches of Penetration Per Year (I.P.Y.) |
| 2                                                                       | 0.0027                                            |
| 3                                                                       | 0.0086                                            |
| 4                                                                       | 0.0076                                            |
| 5                                                                       | 0.0070                                            |
| 6                                                                       | 0.0008                                            |
| 7                                                                       | 0.0057                                            |
| Carpenter 20                                                            | 0.0086                                            |
| No. 20Cb3                                                               | 0.018                                             |
|                                                                         | 0.010                                             |

Table VIII—Continued

CORROSION RATES IN 60% H<sub>2</sub>SO<sub>4</sub> AT 176°F. (80°C.)

| Alloy No. | Losses in Inches of Penetration Per Year (I.P.Y.) |
|-----------|---------------------------------------------------|
| PH55A     | >0.20                                             |
| PH55B     | >0.20                                             |
| PH55C     | >0.20                                             |
| Worthite  | >0.20                                             |
| Illium G  | 0.0039                                            |
| Illium 98 | 0.0048                                            |
| Illium B  | 0.032                                             |

EXAMPLE 7

Comparative tests were conducted in 75 percent sulfuric acid solution at 176°F. Sample discs were prepared and tested in the manner described in Example 2, except that a 75 percent sulfuric acid solution was used in place of the 10 percent sulfuric acid solution. The results of this test are set forth in Table IX.

Table IX

CORROSION RATES IN 75% H<sub>2</sub>SO<sub>4</sub> AT 176°F. (80°C.)

| Alloy No.     | Losses in Inches of Penetration Per Year (I.P.Y.) |
|---------------|---------------------------------------------------|
| 1             | 0.0062                                            |
| 2             | 0.0700                                            |
| 3             | 0.0068                                            |
| 4             | 0.0443                                            |
| 5             | 0.0030                                            |
| 6             | 0.0000                                            |
| 7             | 0.0036                                            |
| Carpenter 20  | 0.050                                             |
| No. 20Cb3     | 0.050                                             |
| PH55A         | 0.15                                              |
| PH55B         | 0.12                                              |
| PH55C         | 0.10                                              |
| 316 Stainless | 1.2                                               |
| Illium G      | 0.028                                             |
| Illium 98     | 0.011                                             |
| Illium B      | 0.026                                             |

EXAMPLE 8

Comparative tests were conducted in 93 percent sulfuric acid solution at 176°F. Sample discs were prepared and tested in the manner described in Example 2, except that a 93 percent sulfuric acid solution was used in place of the 10 percent sulfuric acid solution. The results of this test are set forth in Table X.

Table X

CORROSION RATES IN 93% H<sub>2</sub>SO<sub>4</sub> AT 176°F. (80°C.)

| Alloy No.    | Losses in Inches of Penetration Per Year (I.P.Y.) |
|--------------|---------------------------------------------------|
| 1            | 0.0081                                            |
| 2            | 0.0043                                            |
| 3            | 0.0049                                            |
| 4            | 0.0068                                            |
| 5            | 0.0000                                            |
| 6            | 0.0054                                            |
| 7            | 0.0000                                            |
| Carpenter 20 | 0.024                                             |
| No. 20Cb3    | 0.020                                             |
| PH55A        | 0.045                                             |
| PH55B        | 0.012                                             |
| PH55C        | 0.0006                                            |
| Worthite     | 0.080                                             |
| Illium G     | 0.013                                             |
| Illium 98    | 0.005                                             |
| Illium B     | 0.005                                             |

## EXAMPLE 9

Comparative corrosion tests were conducted at 176°F. in a solution containing 40 percent by weight sulfuric acid and 10 percent by weight nitric acid. Corrosion sample discs were prepared and tested in the manner described in Example 2, except that a 40 percent sulfuric/10 percent nitric acid solution was used in place of a 10 percent by weight sulfuric acid solution. The results of this test are set forth in Table XI.

Table XI

| CORROSION RATES IN<br>40% H <sub>2</sub> SO <sub>4</sub> PLUS 10% HNO <sub>3</sub> AT 176°F. (80°C.) |                                                      |  |
|------------------------------------------------------------------------------------------------------|------------------------------------------------------|--|
| Alloy No.                                                                                            | Losses in Inches of Penetration<br>Per Year (I.P.Y.) |  |
| 5                                                                                                    | 0.0135                                               |  |
| 6                                                                                                    | 0.0130                                               |  |
| 7                                                                                                    | 0.0032                                               |  |

As these results indicate, the alloys of the invention provide very satisfactory corrosion resistance even in environments containing relatively strong oxidizing agents.

## EXAMPLE 10

Comparative corrosion tests were conducted in 10 percent hydrochloric acid at room temperature. Corrosion sample discs were prepared and tested in the manner described in Example 2, except that the test solution was 10 percent hydrochloric acid at room temperature. The results of these tests are set forth in Table XII.

Table XII

| CORROSION RATES IN 10% HCl AT ROOM TEMPERATURE |                                                      |  |
|------------------------------------------------|------------------------------------------------------|--|
| Alloy No.                                      | Losses in Inches of Penetration<br>Per Year (I.P.Y.) |  |
| 1                                              | 0.0122                                               |  |
| 2                                              | 0.0092                                               |  |
| 3                                              | 0.0124                                               |  |
| 4                                              | 0.0111                                               |  |
| 5                                              | 0.0149                                               |  |
| 6                                              | 0.0089                                               |  |
| 7                                              | 0.0111                                               |  |

## EXAMPLE 11

Comparative corrosion tests were conducted in 20 percent hydrochloric acid at room temperature. Corrosion sample discs were prepared and tested in the manner described in Example 2, except that the test solution was 20 percent hydrochloric acid at room temperature. The results of these tests are set forth in Table XIII.

10  
Table XIII

| CORROSION RATES IN 20% HCl AT ROOM TEMPERATURE |                                                      |  |
|------------------------------------------------|------------------------------------------------------|--|
| Alloy No.                                      | Losses in Inches of Penetration<br>Per Year (I.P.Y.) |  |
| 1                                              | 0.0130                                               |  |
| 2                                              | 0.0041                                               |  |
| 3                                              | 0.0046                                               |  |
| 4                                              | 0.0108                                               |  |
| 5                                              | 0.0116                                               |  |
| 10                                             | 0.0019                                               |  |
| 6                                              | 0.0097                                               |  |
| 7                                              |                                                      |  |

The results of the tests of Examples 10 and 11 illustrate that the alloys of the invention are corrosion-resistant even under the highly depassivating influence of solutions such as hydrochloric acid.

In view of the above, it will be seen that the several objects of the invention are achieved and other advantageous results attained.

As various changes could be made in the above products without departing from the scope of the invention, it is intended that all matter contained in the above description shall be interpreted as illustrative and not in a limiting sense.

What is claimed is:

1. A corrosion-resistant alloy consisting essentially of between about 35.2 and about 46.2 percent by weight nickel, between about 14.9 and about 25.3 percent by weight chromium, between about 6.7 and about 14.5 percent by weight molybdenum, between about 4.3 and about 8.1 percent by weight copper, between about 14.06 and about 30.62 percent by weight iron, up to about 0.11 percent by weight carbon, up to about 1.00 percent by weight silicon, up to about 1.50 percent by weight manganese, up to about 0.010 percent by weight boron, up to about 1.00 percent by weight niobium, up to about 2.00 percent by weight tantalum, and up to about 1.00 percent weight titanium, the sum of the molybdenum content and the copper content being at least about 11.7 percent by weight and the sum of the niobium content and one-half of the tantalum content being no greater than about 1.00 percent by weight.
2. An alloy as set forth in claim 1 wherein the sum of the niobium content and the tantalum content is at least about 10 times the carbon content.
3. An alloy as set forth in claim 1 wherein the titanium content is at least about five times the carbon content.
4. An alloy as set forth in claim 1 wherein the nickel content is between about 35.70 and about 46.17 percent by weight, the chromium content is between about 18.19 and about 25.28 percent by weight, the molybdenum content is between about 6.74 and about 9.66 percent by weight, the copper content is between about 4.37 and about 7.01 percent by weight, the titanium content is between about five times the carbon content and about 1.00 percent by weight, the sum of the tantalum and niobium content is between about ten times the carbon content and about 1.00 percent by weight, and the sum of the molybdenum and copper content is between about 11.7 percent and about 16.67 percent by weight.

\* \* \* \* \*